

## UNITED STATES PATENT OFFICE

2,640,016

## MANUFACTURE OF COKE

Samuel W. Martin, Chicago, Ill., assignor to  
 Great Lakes Carbon Corporation, New York,  
 N. Y., a corporation of Delaware

No Drawing. Application August 31, 1950,  
 Serial No. 182,634

4 Claims. (Cl. 202—33)

1

This invention relates to novel compositions suitable for coke manufacture and to processes for coking such compositions. More particularly, this invention relates to compositions comprising caking coals and petroleum coke having properties which peculiarly render such coke of high utility when blended with caking coals in coke manufacture.

In accordance with well accepted and standardized practices, blast furnace and metallurgical grade cokes are prepared by the carbonization of various caking coals. Coking is effected by heating a caking coal or mixtures of various types of caking coal in a slot or beehive oven at temperatures up to 1204° C. during a 18 to 30 hour cycle. From an economy standpoint it is desirable to select and utilize the so-called high volatile caking coals. However, it is known to those skilled in the art that very few so-called high volatile caking coals are available which can produce satisfactory blast furnace or foundry grade coke without the blending of such coals with so-called low volatile coals of the Pocahontas type. Cokes prepared from the high volatile coals do not have sufficient hardness and strength and have a tendency to degrade and produce fines in handling. The so-called low volatile caking coals are blended with the high volatile coals to increase the surface hardness of the coke and thereby increase resistance of the coke to abrasion. As previously mentioned, the addition of low volatile caking coals to carbonaceous compositions intended for coke manufacture may be quite costly, this often being due to the geographical location of such coal deposits with respect to the coke manufacturer. In addition, the low volatile caking coals continue in high demand and in rather short supply, this being partially due to the rigid specifications which have been placed on such a material.

As a substitute for the low volatile caking type coals, the use of "low temperature char" has been suggested and has met with some success. However, this type of additive varies in its properties and specifications, nor has a constant supply of this material been assured coke manufacturers. The use of petroleum coke has also been suggested as a component for coke manufacture. Petroleum cokes having a volatile content of 8 to 13% have been admixed with high volatile caking coals followed by subjecting this mixture to carbonization. These attempts have been commercially unsuccessful, the probable reasons for which will be subsequently pointed out herein.

It is an object of this invention to provide a

2

novel composition well adapted to the manufacture of hard, dense, strong metallurgical coke.

It is a further object of the invention to provide a coke suitable for metallurgical, foundry and blast furnace practice and a process for its manufacture.

It is a further object of this invention to provide a raw material of uniform composition suitable for the manufacture of metallurgical and blast furnace coke.

It is still a further object of the invention to provide a process for the manufacture of a hard, dense coke having uniform physical properties.

It is still a further object of the invention to provide a process for the manufacture of blast furnace and foundry coke which obviates the use of and necessity for low volatile caking coals.

It is an additional object of the invention to provide a blast furnace or foundry coke having a reduced ash content.

The above objects, as well as others which will become apparent upon an understanding of the invention as hereinafter described, are realized by preparing a composition comprising a mixture of caking coal and petroleum coke. The petroleum coke component has a volatile content of about 14-35% by weight and is further characterized by its ability to form a hard, dense agglomerate on being heated at a temperature of about 950° C. to substantially remove the volatile matter of the coke.

The petroleum coke or petroleum carbon which I employ in admixture with caking coals is produced by the non-catalytic pyrolysis of petroleum hydrocarbons, the latter including topped crude oils, thermally cracked petroleum residuums and/or recycle stocks from the thermal or catalytic cracking of petroleum fractions. The non-catalytic cracking of petroleum hydrocarbons involves the heating of particular petroleum fractions or components to a temperature of between about 412° to 490° C. The petroleum cokes thus produced which I have found to be useful in the present invention have a volatile content of about 14 to about 35% by weight, this "volatile content" being determined in accordance with the A. S. T. M. Procedure No. D271-48 as modified for peat and lignite, and being exclusive of water. In accordance with this procedure, a relatively small sample of petroleum coke is heated at 950° C. for a period of time between about 5 to 10 minutes. The difference in weight of the sample prior to and after heating constitutes the "volatile content" of the coke. I have found that

55 there are distinct and highly important differ-

ences between petroleum cokes having the same volatile content, and I have further found that only those petroleum cokes having a volatile content within the aforementioned range and which, in addition, form a hard, dense coke agglomerate while being heated in accordance with the previously mentioned A. S. T. M. procedure, or at a temperature of 950° C., are suitable for my purposes. As will be subsequently illustrated herein neither petroleum cokes having a volatile content less than about 14% nor cokes having a volatile content between 14 and 35% which will not "agglomerate" or form a hard, dense "button" are suitable for the purposes of this invention.

In a specific embodiment of my invention, a major portion of a high volatile caking coal is blended with a minor portion of petroleum coke, the latter having a volatile content of about 14 to about 35% by weight and being further characterized by its ability to form a hard, dense agglomerate on being heated at a temperature of about 950° C. to substantially remove the volatile matter, are intimately blended and crushed or ground so that a major portion and preferably 60% of the mixture, will pass through an  $\frac{1}{8}$ " screen. This mixture is then heated in a slot oven to a temperature of 982° to 1080° C. for a period of about 30 to 18 hours. The resulting coke is found to be equivalent to a coke prepared from a high volatile caking coal in admixture with a minor portion of a low volatile or Pocohontas type caking coal.

Slot ovens or by-product ovens are well-known in the art. These ovens are elongated, narrow, vertical chambers which are heated from the sides. A deep vertical bed of the material to be coked is placed in the slot oven and is then coked by virtue of indirect heating through the walls.

In a further embodiment of my invention I prepare a composition comprising a major portion of high volatile caking coal together with minor portions of a low volatile caking or Pocohontas type coal and petroleum coke having the previously described properties or characteristics. The ratios of petroleum coke to low volatile caking coal may be adjusted to meet the specifications of the coke manufacturers, but in any event the total amount of low volatile caking coal plus the petroleum coke will generally and preferably be less than the amount of high volatile caking coal in the mixture.

While I may employ a petroleum coke having a volatile content of about 14 to 35% by weight, which coke in addition will have the agglomerating properties described herein, I find it to be preferable to employ a coke having a volatile content of between about 16 and about 20% by weight. It will be apparent to those skilled in the art that these ranges of volatile content may and often do include minor amounts of petroleum coke having a volatile content falling outside of this range. While the improvements described herein can be obtained by the utilization of such materials, I have found it to be distinctly preferable to select a petroleum coke wherein all of the coke has a volatile content between 14 and 35% by weight and preferably between 16 to 20% by weight.

In order to more fully illustrate the nature and character of my invention, but with no intention of being limited thereby, the following specific examples are set forth. In all of these examples, the cokes were prepared by heating a mixture of the indicated components, 60% of which mixture would pass a  $\frac{1}{8}$ " screen, to a temperature of 982° to 1080° C. for a period of time varying between 18 to 24 hours. The resulting cokes are evaluated by their shatter, tumbler hardness (% +1") and tumbler stability (% + $\frac{1}{4}$ ") values. The shatter and tumbler tests were conducted in accordance with A. S. T. M. procedures Nos. D141-48 and D249-29 respectively. The volatile matter (water free) was determined in accordance with the previously mentioned A. S. T. M. procedure.

In the examples set forth in Table I, a rather weakly caking high volatile coal (38 to 40% V. M.) was employed as a major component. This was intimately mixed with a low volatile coal (16 to 20% V. M.) and two petroleum cokes, one having a volatile content of 12% and which was of the "non-agglomerating" type and one having a volatile content of 18% and which agglomerated when heated at 950° C. to form a hard, dense "button" which would support a weight of two to three pounds or more. Acceptable values for shatter and tumbler for a coke prepared from this type of high volatile coal are indicated in the appropriate columns in the "Control" examples.

Table I

| Example No. | Percent H. V. Coal | Percent L. V. Coal | Percent Pet. Coke | Percent Vol. Pet. Coke | Shatter, Percent + 2" | Tumbler, Percent + 1" | Tumbler, Percent + $\frac{1}{4}$ " |
|-------------|--------------------|--------------------|-------------------|------------------------|-----------------------|-----------------------|------------------------------------|
| Control     | 90                 | 10                 |                   |                        | 43.8                  | 33                    | 70                                 |
| Control     | 85                 | 15                 |                   |                        | 49.2                  | 32                    | 71                                 |
| 1           | 90                 |                    | 10                | 12                     | 45                    | 21                    | 57                                 |
| 2           |                    |                    | 15                | 12                     | 39                    | 30                    | 60                                 |
| 3           |                    |                    | 10                | 18                     | 49                    | 30                    | 71                                 |
| 4           |                    |                    | 15                | 18                     | 52                    | 32                    | 70                                 |
| 5           | 85                 |                    | 20                | 18                     | 50                    | 42                    | 70                                 |
| 6           | 80                 | 10                 | 10                | 18                     | 51                    | 31                    | 71                                 |

In a further embodiment of my invention, a mixture of 95 to 75% by weight of high volatile caking coal and 5 to 25% by weight of petroleum coke is prepared and comminuted such that a major portion and preferably at least 60% of the mixture will pass through an  $\frac{1}{8}$ " screen. The petroleum coke should preferably have a volatile content of about 16 to about 20% by weight and it is further characterized by its ability to form a hard, dense agglomerate on being heated at a temperature of about 950° C. to substantially remove the volatile matter.

It is apparent from the above results that a coke prepared from a mixture of high volatile coal and petroleum coke having a volatile content of 12% by weight falls considerably short of acceptance for blast furnace coke. On the other hand, the use of petroleum coke having a volatile content of 18% and which will "agglomerate" on heating to 950° C. equals, and in some instances, surpasses the minimum desired specifications.

In the following examples it was desired to prepare a coke suitable for blast furnace opera-

tion which would match a coke prepared from a high volatile caking coal and a medium volatile Pocohontas type coal. For illustrative purposes, two petroleum cokes were selected having volatile contents of 13 and 16% by weight, neither of which would "agglomerate" when heated at 950° C. in accordance with procedures previously described herein. The shatter and tumbler figures for the "Control" examples indicate acceptable values in this particular instance.

Table II

| Example No. | Percent H. V. Coal | Percent Med. Vol. Poco-hontas | Percent Pet. Coke | Percent Vol. Pet. Coke | Shatter, Percent + 2" | Tumbler, Percent + 1" | Tumbler, Percent + 1/4" |
|-------------|--------------------|-------------------------------|-------------------|------------------------|-----------------------|-----------------------|-------------------------|
| Control...  | 90                 | 10                            |                   |                        | 51                    | 39                    | 69                      |
| 7-----      | 90                 | 10                            | 13                | 13                     | 37                    | 27                    | 65                      |
| Control...  | 80                 | 20                            |                   |                        | 58                    | 47                    | 67                      |
| 8-----      | 80                 | 20                            | 13                | 13                     | 48                    | 39                    | 61                      |
| 9-----      | 90                 | 10                            | 16                | 16                     | 45                    | 25                    | 65                      |
| 10-----     | 80                 | 20                            | 16                | 16                     | 40                    | 35                    | 60                      |

The above results indicate that petroleum coke having a 13% volatile content is an inferior additive to high volatile caking coals for the manufacture of blast furnace coke as is a 16% volatile content petroleum coke which will not "agglomerate" upon heating to 950° C. It was subsequently indicated that the 16% V. M. coke contained a substantial amount of oily material which was removed during the volatile content A. S. T. M. test and which could also be removed merely by heating the petroleum coke to a temperature of 400° to 500° C.

In the example set forth in Table III, petroleum cokes having several volatile contents, and all of which "agglomerated" on heating to 950° C., were mixed with a high volatile caking coal (38% V. M.) in the indicated amounts. The shatter and tumbler (+ + 1/4") properties were determined, values of +50 and +60 respectively being a minimum requirement for this particular coke.

Table III

| Example No. | Pet. Coke, Percent Volatile | Pet. Coke in Mixture | Shatter, Percent + 2" | Tumbler, Percent + 1/4" |
|-------------|-----------------------------|----------------------|-----------------------|-------------------------|
| 11-----     | 17                          | 10                   | 61                    | 72                      |
| 12-----     | 17                          | 20                   | 60                    | 71                      |
| 13-----     | 22                          | 10                   | 62                    | 72                      |
| 14-----     | 22                          | 20                   | 64                    | 72                      |
| 15-----     | 30                          | 10                   | 60                    | 71                      |
| 16-----     | 30                          | 20                   | 64                    | 70                      |
| 17-----     | 35                          | 10                   | 52                    | 71                      |
| 18-----     | 35                          | 20                   | 54                    | 70                      |

I have thus shown that by selecting a petroleum coke having certain properties and blending such a coke with high volatile caking coals and/or low volatile caking coals, I have been able to produce metallurgical grade and blast furnace coke of a quality comparable to or superior to cokes prepared in accordance with conventional prac-

tice, i. e. by the blending of high volatile and low volatile caking coals.

The above examples have been recited by way of illustration and not limitation.

5 Having thus completely described the nature and character of the invention, I claim:

1. A process for manufacturing metallurgical coke which comprises forming an intimate mixture consisting essentially of caking coal at least 10 a major portion of which is of the high volatile

type, and five to twenty-five per cent of petroleum coke, the major portion of the particles of said mixture passing a  $\frac{1}{8}$  inch screen, forming a deep bed of the mixture in a narrow, vertical coking zone, coking the mixture by indirect heat at a temperature of about 982° to 1204° C., said petroleum coke consisting essentially of coke having a volatile content in the range of 14% to about 35% by weight as determined by A. S. T. M. procedure No. D271-48 as modified for peat and lignite, and exclusive of volatile material evolved at temperatures of 400-500° C., and further characterized by forming a dense, hard, agglomerated coke when heated according to said procedure.

2. The process of claim 1 wherein the volatile content of said coke is about 16% to about 20% by weight.

3. The process of claim 1 further characterized in that the mixture contains 95% to 75% of high volatile caking coal.

4. The process of claim 1 further characterized in that the coal is a mixture of a major portion of high volatile caking coal and a minor portion of a low volatile caking coal, the quantity of high volatile caking coal being in excess of the total proportion of low volatile caking coal plus the petroleum coke.

50 SAMUEL W. MARTIN.

References Cited in the file of this patent

UNITED STATES PATENTS

55 Number Name Date  
1,815,918 Knowles July 28, 1931

OTHER REFERENCES

Chemistry and Industry, vol. 51, No. 22, May 60 27, 1932 pages 467-469, "Petroleum Coke," by Morrell et al.

Industrial and Engineering Chemistry, vol. 36, No. 12, December 1944, pages 1140-1144, "Petroleum Coke" by Berry et al. (Copies available in 65 Scientific Library.)